

J. A. E. CRISWELL.  
METHOD OF MAKING MATCHES.  
APPLICATION FILED SEPT. 3, 1908.

988,254.

Patented Mar. 28, 1911.

4 SHEETS—SHEET 1.



Vitneess:  
Julius Koch  
E. Kramer

Inventor  
John E. Criswell,  
By his Attorney  
Criswell Criswell

J. A. E. CRISWELL,  
METHOD OF MAKING MATCHES,  
APPLICATION FILED SEPT. 3, 1908.

988,254.

Patented Mar. 28, 1911.

4 SHEETS-SHEET 2.



Witnesses:  
Julian E. Criswell  
E. Fransen

Inventor  
By his Attorney  
J. A. E. Criswell  
Criswell Criswell.

J. A. E. CRISWELL,  
METHOD OF MAKING MATCHES,  
APPLICATION FILED SEPT. 3, 1908.

988,254.

Patented Mar. 28, 1911

4 SHEETS—SHEET 3.



*John A. E. Criswell  
6/28/08*

Inventor  
John A. E. Criswell  
By his Attorney  
Criswell & Criswell

J. A. E. CRISWELL.  
METHOD OF MAKING MATCHES.  
APPLICATION FILED SEPT. 3, 1908.

988,254.

Patented Mar. 28, 1911.

4 SHEETS—SHEET 4.



Fig. 9.



Fig. 10.

Witnesses:

*Julian L. E. Knauss*

Inventor  
J. A. E. Criswell  
By his Attorney  
Criswell Criswell

# UNITED STATES PATENT OFFICE

JAMES A. EKIN CRISWELL, OF NEW YORK, N. Y.

## METHOD OF MAKING MATCHES.

988,254.

Specification of Letters Patent. Patented Mar. 28, 1911.

Application filed September 3, 1908. Serial No. 451,515.

To all whom it may concern:

Be it known that I, JAMES A. EKIN CRISWELL, a citizen of the United States, and a resident of New York, borough of Brooklyn, county of Kings, and State of New York, have invented certain new and useful Improvements in Methods of Making Matches, of which the following is a full, clear, and exact description.

10 This invention relates to matches and the method of making match splints, and more particularly to forming round splints from material a part or whole of which is in a plastic or semi-plastic state.

15 The primary object of the invention is to provide a system in which material ordinarily going to waste or used for other purposes may be utilized to make matches.

Other objects are to provide a system in 20 which there is a large output of splints with a minimum of waste and in which finished splints of various shapes may be produced and which may be of one or a series of colors as desired, and to provide a system in 25 which the splints may be made of a uniform quality and with sufficient rigidity and strength to materially reduce their liability to break while using, and at the same time produce splints that will ignite and burn 30 properly.

A further object of the invention is to provide composite matches in each of which there will be a strengthening body and which will be attractive in appearance.

35 The invention will be hereinafter more particularly described with reference to the accompanying drawings which form a part of this specification, and will then be pointed out in the claims at the end of the description.

40 In the drawings, Figure 1 is a side elevation, partly in section and partly diagrammatic, of one means for carrying the invention into practice. Fig. 1<sup>a</sup> is a plan view of one set of rolls which may be utilized in carrying out my method. Fig. 2 is an enlarged elevation, partly in section and partly diagrammatic, of part of the apparatus shown in Fig. 1. Fig. 2<sup>a</sup> is an enlarged 45 fragmentary elevation of one form of device for forming the material into splints. Fig. 3 is a side elevation of one form of machine for making one or more of the outer layers. Figs. 4 and 5 are diagrammatic views showing how various layers and kinds of layers may be united. Fig. 6 is an end

view of still another form of series of layers. Fig. 7 shows the layers in Fig. 6 after being formed or partly formed into splints: Fig. 8 is a detail perspective view of one of the 60 finished matches. Fig. 9 shows how one of the layers may be caused to pass through a liquid before being united with the other layers; and Fig. 10 is an elevation of means for assisting in arranging the fibers, strands 65 or filaments of material that does not require to be cut or shredded as it enters the apparatus.

The tank 10, Fig. 3, contains a wood-pulp stock from which a layer or web is made. 70 The pulp is collected by the cylinder 11 from which it is couched by a roll 12 on to the apron or felt 13 as is usual in paper making machines, and then passes between the rolls 14 which forces some of the moisture out of the web or layer 15. As shown two layers 16 and 16<sup>a</sup> of this wet pulp of the proper thickness is formed, and either or both are fed from reels 17 on which it has been previously rolled. The layer of pulp 80 16<sup>a</sup> has fine dry powder as flour or starch, blown over its surface from a receptacle 18 by means of a fan 19, and both layers 16 and 16<sup>a</sup> pass between the rolls 20 forming a preliminary compressing and splint-forming 85 device. A layer 21 of wood, straw or bagasse, prepared as hereinafter explained is fed direct over the drum or cylinder 22 between the latter and a roll 23 on to a traveling apron 24. The layer 21 has a suitable adhesive substance as powdered flour or starch supplied to and scattered over its surface from a receptacle 25. The three layers are of such a thickness that when properly compressed they make a composite 90 layer of just the thickness of the splints. The layers 16, 16<sup>a</sup> and 21 as they pass between the rolls 20 will be pressed together and the adhesive substance between the layers will cause them to form a composite 95 layer or web of splints. The rolls 20 are fluted or grooved, Fig. 2, and besides forming the composite layer they also partially form the layer into splints. This web passes through a second compressing device 26. 100 The device 26 comprises two grooved rolls 27 similar to rolls 20, which are adapted to complete compressing the material into the shape of finished long splints as best shown in Fig. 2<sup>a</sup>. If not entirely severed from 11 each other the splints pass between a cutting device 28 of a match-making machine such

as shown in my Patent No. 656,014, dated August 14, 1900, or my Patents 716,810, 716,815, and other of my patents issued December 23, 1902. As shown the cutting device 5 consists of a metallic roll 29 and a series of cutters 30 spaced the width of the splints on a spindle 31 and after being cut pass through a separator 32 to divide them into independent rows, and are then cut by 10 a cutter bar 33 while in a suitable frame or holding means 34 as in my patents previously mentioned. The splints are thus formed with a strengthening core 35 and an outer coating 36.

15 The layer 21 when consisting in part or in whole of strands or filaments as best shown in cross-section in Fig. 2<sup>a</sup> and where such filaments or shreds are cut or made from material that is larger than is suitable for 20 splints or as a part of said layer, the wood, bagasse, straw and similar material is subjected to the action of the sets of rolls 39, 40 and 41 as shown in Figs. 1 and 1<sup>a</sup>. The wood or other material is fed inward by a 25 traveling apron 42 over a table 43 to the set of cutting rolls 39. These rolls have annular and V-shaped cutting devices 44 which cut the material in the direction of its feed and these strands, strips and particles are 30 caused to pass to the second set of rolls 40. These rolls have peripheral ribs or teeth 45 that extend transversely of the travel of the material and are adapted to break the strands or shreds somewhat and to better assist 35 in forming a proper layer, from which the material passes to the smooth rolls 41 that form the material into a better and compact layer of the desired thickness, before passing around the drum or cylinder 22, 40 a pan 46 being provided beneath the shredding rolls to catch any material that might pass beneath said rolls.

45 The layer 16<sup>a</sup> instead of passing from a reel as in Fig. 2 is shown as passing around the pulleys 47 and as being formed by several layers or webs 48 that are pressed together by the rolls 48<sup>a</sup>. Two of these webs have a suitable adhesive substance as flour or starch blown over their surfaces from the 50 hoppers 49, a blower 50 being provided for this purpose as already explained. The splints after passing the rolls 27 and before reaching the match machine, if not sufficiently dry, pass through a suitable device 55 55 to dry the splints whether still joined together by a film or not, and the splints are finished by hand, or automatically as in my patents before mentioned. The carrier 52 of the machine 52<sup>a</sup> takes the splints and 60 forces the same into a dipping carrier 53 as in my Patent 716,815. The dipping carrier 53 passes around suitable pulleys to the paraffin and composition apparatus 54 around the pulleys 55 back to the machine 65 to again receive splints. Before returning

to the machine the completed splints are ejected from the dipping carrier by the ejecting plungers 56 and are received by a conveyer 57 in substantially the same manner as in my Patent 716,810, before referred to.

70 The method and operation of the apparatus will be readily understood from the foregoing description when taken in connection with the accompanying drawings. 75 The layers of wet pulp 16 and 16<sup>a</sup> after being formed on a cylinder and couched to the felt or run from the apron on to the wire and couched to the felt of a suitable paper making machine such as a Fourdrinier or a 80 modification of the same or otherwise is caused to pass with the intermediate layer 21 of strengthening fiber or shredded wood, bagasse, straw, etc., between the rolls 20. The corrugated composite layer passes 85 between the splint-forming device 25 and from there through a drier 51 if necessary, and then to a match-making machine and the matches completed as disclosed in my patents referred to or in the usual or in any 90 preferred manner.

95 While I have described certain means for carrying the invention into practice it will be understood that various means, apparatus or combinations may be employed for this purpose, and that the layers may be of any suitable material and may be arranged in various ways with respect to each other. In Fig. 4 the fibrous material or layer 21 may be fed to the layer of pulp while on the 100 felt or apron 13. This layer may be then used or in combination with others to make the splints. The intermediate layer 37 shown in Fig. 5 is a veneer of wood or may be a web of paper or paper board, and this 105 layer 37 is combined with the layers 16 and 16<sup>a</sup> and may be formed into splints in substantially the same manner as already described. The central layer 38 in Fig. 6 is 110 of independent cores of any suitable shape and material. The outer layers are also of any suitable material as pulp and preferably have some adhesive substance between them so that when passed between rolls in the manner indicated they will be formed 115 into independent splints or splints held together with a thin film as in Fig. 7. In this latter case the splints are made into complete splints as already described or in any 120 preferred way.

125 The material may be first made in a sheet or strip form and then if necessary softened to make the matches. As one means for this purpose the device shown in Fig. 9 may be employed. The layer 58 before reaching the splint-forming rolls is caused to pass around pulleys 59 and in contact with a liquid, as water, in a pan or receptacle 60 and then around pulleys to the splint-forming device.

In Fig. 10 is shown one means for arranging the long fibers of previously shredded material or such as has threads or filaments. The large drum or cylinder 61 has a series of peripherally spaced serrated and circular plates 62, adjacent to which rotate the smaller cylinders 63 with similar serrated plates only a portion of the serrated surface being shown. The material in passing between the several drums or cylinders has the threads properly arranged lengthwise of the layer preparatory to its proper formation or compression. The device shown is like certain features of a carding engine.

If desired, one layer may be made of one color and another or the others of the same or of different colors and these may be colored at any suitable stage of the process so that the finished splints will be differently colored. The cheapest kind of material may be used as a filler or to make the entire splints and to make the parts adhere better any suitable adhesive or glutinous substance may be added at any suitable stage of the process. A device such as shown in Fig. 9 might be employed for this purpose.

In practice it is intended to use excelsior, sawdust, shavings, straw, seaweed, old paper, fiber of any suitable kind or other material which in many instances go to waste. These or any of the material employed may be macerated and may be chemically or mechanically treated as by boiling or bleaching or otherwise treated with or without chemicals or other ingredients mixed therewith to make them suitable for use in the manufacture of matches.

Where the material is of such a nature as to require it, paraffin or other inflammable substances may be added before the layers are compressed into splints, or the paraffin or like material may be added at any step in the manufacture or the splints may be dipped and treated as usual; and where cotton or such fiber mixed or not with other material is used to form a layer, it may be treated with a suitable chemical to prevent glowing. A device such as shown in Fig. 9 also might be employed for this purpose.

The pressure or other means used in forming the splints is regulated so as to avoid having the splints too compact for treatment to complete the matches or to destroy the qualities necessary to a free burning and strong match, and any suitable means or material may be employed to increase the homogeneity of the splints.

The layers may be fed from reels where the material will permit, and any suitable number of layers may be employed.

Instead of the several sets of splint forming rolls being employed, the splint-forming and compressing rolls 26 might be substituted in the first instance, and in any case where it is desirable the splints may be

caused to pass between rolls or other polishing means.

While reference has been made particularly to round matches it will be understood that these may be of any desired shape, and may be made, cut or formed in any desired manner.

By "shredded material" or "shredded woody material" is intended to mean wood proper, bagasse, straw, or other material that is not first reduced to pulp and that contains threads, filaments, or strands, united or not with other material and that is adapted to give strength and rigidity to the wood pulp or layers of pulp.

It will be seen from the foregoing that a strong and efficient match is produced, and each splint may be provided with a central strengthening core and an outer coating. It will be seen also that the splints may be made of any suitable form and in very large quantities with very little waste and with the possibility of turning out poor splints or splints that are not uniform in size and quality reduced to a minimum, at the same time permitting the utilization in the manufacture of matches of cheap material and material that ordinarily goes to waste or is burned for lack of other means of disposition.

Having thus described my invention, I claim as new and desire to secure by Letters Patent:

1. In the manufacture of matches, the method which consists in taking two independent soft layers of wood pulp, interposing between the two layers of pulp a layer or web of shredded woody material having threads or strands extending lengthwise of the web and adapted to form a strengthening and stiffening body to the wood-pulp layers, uniting the combined layers together under pressure and simultaneously forming splints as the layers are combined.

2. The method of making matches, which consists in forming a layer of shredded wood material having long fibrous threads or strands arranged lengthwise of the layer, and uniting with the woody strands of wood material wood pulp, and forming the splints from the combined strands and pulp whereby the said strands may serve to strengthen and stiffen the splints for the purpose set forth.

3. The method of making matches, which consists in collecting wood pulp and forming two wet layers of the same, interposing a layer of long fibrous material between the two layers of the pulp, and then forming splints from the combined layers to provide a strengthening core for each splint, for the purpose set forth.

4. The method of making matches, which consists in collecting wood pulp and forming two wet layers of the same, interposing

a layer of long fibrous material with its fiber extending lengthwise of the layer between the two layers of pulp, and subjecting the combined layers to pressure to form splints each 5 of which has a strengthening core substantially as and for the purpose described.

5. The method of making matches, which consists in forming one or more sheet-like layers of wood pulp, distributing a layer of 10 fibrous material on to the pulp and while the pulp is in a soft or wet state subjecting the combined layers to pressure to form splints, separating the splints and then holding the splints for treatment to complete the 15 matches.

6. In the manufacture of matches, the combination of independent soft layers of wood pulp and intermediate fibrous or shredded woody material having threads or 20 strands extending lengthwise of the web and adapted to form a strengthening and stiffening body to the wood pulp layers, the combined layers of material being united together under pressure thus forming splints.

7. In the manufacture of matches, the method which consists in uniting wood that has not been reduced to pulp, and wood pulp, forming a web of match splints therefrom by compressing the pulp and the wood, 30 and cutting the web.

8. The method of making matches, which consists in collecting wood pulp and uniting with it an independent layer of fibrous material, and forming a web of match splints 35 therefrom by compression and while the pulp is soft so that each splint will have an inner core and an outer casing or cover.

9. The method of making matches, which consists in uniting material having long 40 woody fibers, and wood pulp, and forming a web of match splints therefrom by compres-

sion and while the pulp is soft so that each splint will have an inner body of the fibrous material and an outer cover or casing of the pulp.

45

10. In the manufacture of matches, the method which consists in taking two independent soft sheet-like layers of wood pulp, interposing between the two layers of pulp a layer or web of shredded woody material 50 having threads or strands extending lengthwise of the web and adapted to form a strengthening and stiffening body to the wood-pulp layers, uniting the combined layers together under pressure and simultaneously forming splints as the layers are combined.

11. In the manufacture of matches, the method which consists in forming a sheet-like layer of shredded woody material having long fibrous threads or strands arranged lengthwise of the layer, and uniting with the woody strands of woody material wood pulp, and forming the splints from the combined strands and pulp whereby the said 65 strands may serve to strengthen and stiffen the splints for the purpose set forth.

12. In the manufacture of matches, the method which consists in taking long strands or filaments of a fibrous material, 70 uniting wood pulp with the strands, and forming a web of match splints with the strands extending lengthwise of the match bodies whereby said bodies are strengthened, 75 and then cutting the web into match splints.

This specification signed and witnessed this second day of September A. D. 1908.

JAMES A. EKIN CRISWELL.

Witnesses:

M. TURNER,  
A. REDMOND.